

# UNITED STATES PATENT OFFICE.

WILBUR B. DRIVER, OF EAST ORANGE, NEW JERSEY.

## ALLOY FOR RESISTANCE ELEMENTS, &c.

1,274,250.

Specification of Letters Patent. Patented July 30, 1918.

No Drawing.

Application filed January 2, 1914. Serial No. 810,012.

To all whom it may concern:

Be it known that I, WILBUR B. DRIVER, a citizen of the United States, residing at East Orange, Essex county, New Jersey, have invented certain new and useful Improvements in Alloys for Resistance Elements, &c., of which the following is a full, clear, and exact description.

My invention relates to a new and improved alloy for resistance elements, etc., and has for its object to produce an alloy which has a high specific electrical resistance together with a prolonged life under conditions of high temperature, so as to render it suitable for the making of resistance elements.

My invention is based on the discovery that when titanium in substantial amounts is added to other metals, such as nickel, iron, copper, etc., or alloys of metals, it causes a marked increase in specific electrical resistance of the alloy so formed and produces an alloy which is extremely resistant to oxidation, especially at high temperatures. From numerous experiments I have found that titanium is more powerful in these respects than chromium, and that titanium and chromium when simultaneously used as alloys with other metals, produce highly desirable results. I have also discovered that relatively large quantities of titanium can be used in alloys without making them too hard or too brittle to allow rolling and drawing.

For the purpose of illustration I give below a list of alloys made according to my invention, together with the specific electrical resistance in microhms per cubic centimeter of said alloys respectively.

|             | Nickel. | Chromium. | Titanium. | Iron. | Manganese. | Specific resistance. |
|-------------|---------|-----------|-----------|-------|------------|----------------------|
| No. 1.....  | 75%     | 10%       | 6%        | 19%   | 2%         | 77                   |
| No. 2.....  | 68      | 10%       | 4         | 11    | 2%         | 117                  |
| No. 3.....  | 65      | 8         | 5         | 27    |            | 90                   |
| No. 4.....  | 65      | 6         | 6         | 19    | 10         | 106                  |
| No. 5.....  | 60      | 12        | 12        | 24    | 5          | 112                  |
| No. 6.....  | 60      | 12        | 6         | 19    | 3          | 126                  |
| No. 7.....  | 40      | 15        | 6         | 39    |            | 113                  |
| No. 8.....  | 20      | 10        | 6         | 54    |            | 117                  |
| No. 9.....  | 20      |           | 6         | 64    |            | 100                  |
| Copper.     |         |           |           |       |            |                      |
| No. 10..... | 80      | 10%       | 8         | 7     |            | 48                   |
| No. 11..... | 75      | 8         | 8         | 17    |            | 57                   |
| No. 12..... | 45      | 65        | 3         | 7     |            | 77                   |
| No. 13..... | 94      |           | 5         | 1     |            | 22                   |

The percentages in the above table, while

not exact, are approximately correct. The presence of titanium in each of these alloys increases the life at high temperatures of the metal or alloy to which it is added.

The qualities imparted by the addition of titanium are particularly valuable in connection with resistance elements used in electrical apparatus such as heaters, toasters and cooking appliances, where the resistance elements are subjected to high temperatures by the passage of electric currents through them. These electrical resistance elements may be of any ordinary form, such for instance as open helices or spirals. The form of the resistance element constitutes no part of my invention.

I have discovered that titanium hardens the metals or alloys to which it is added so that the quantity of titanium that can be used is limited when it is necessary to retain such malleability and ductility as will permit the rolling or drawing of the alloy. The alloys above referred to are all sufficiently malleable and ductile so as to permit such rolling and drawing.

The melting to form the alloy can be carried on in any approved manner, special care being exercised to prevent the introduction of carbon, either through the metals that are used or through contamination from the vessel in which the melting is done. Pure titanium is not commercially obtainable so far as I am aware. My experiments have been carried out with nickel-titanium and ferro-titanium. Even if pure titanium were available its melting point is so high that it would not be desirable to form an alloy directly from it. An alloy of one of the metals which is to form a substantial part of the final alloy should be used as a carrier for the titanium for the final melting, which is as low as possible in contained titanium as is compatible with the amount of titanium to be introduced, thereby providing a low melting point and making easier its incorporation into the final alloy. Owing to the relatively low specific gravity of titanium, there is a tendency of the titanium carrying alloy to rise to the surface of the melted bath, and care should be used to make sure that it is entirely submerged so that it will be properly incorporated into the bath.

Quantities of titanium as low as one per cent. (1%) are effective in increasing the electrical resistance of alloy containing it

and in protecting the alloy against oxidation at high temperatures. This effect increases with the percentage of titanium added. The only use of titanium in connection with melted metal baths of which I am aware, has been for the purpose of cleansing steel by removing impurities therefrom, and in this connection only small fractions of one per cent. (1%) have been found necessary or desirable. So far as I am aware, the quantity so used has been limited to less than one-half of one per cent., so that in the finished product there remains no substantial amount of titanium and no amount which affects in any substantial degree the specific electrical resistance, life or hardness of the ultimate product.

As will be evident to those skilled in the art, the employment of my invention permits of considerable modification and variation without departing from the spirit of my invention or the scope of the appended claims.

What I claim is:

1. A ductile and malleable alloy of high specific electrical resistance containing as a constituent at least one per cent. of titanium and over twenty per cent. of nickel, substantially as described.

2. A ductile and malleable alloy containing as a constituent at least one per cent. of titanium and over twenty per cent. of nickel, substantially as described.

3. A ductile and malleable alloy containing as constituents over twenty per cent. of nickel and at least one per cent. of titanium, substantially as described.

4. An electrical resistance element consisting of a ductile and malleable alloy containing as constituents nickel and at least one per cent. of titanium, substantially as described.

5. A ductile and malleable alloy of high specific electrical resistance containing titanium as a constituent and over twenty per cent of nickel, the titanium being sufficient in amount to produce high electrical resistance and greatly retard oxidation at high temperatures.

6. An electrical resistance element comprising a ductile and malleable alloy containing as constituents over twenty per cent. of nickel and at least one per cent. of titanium, substantially as described.

WILBUR B. DRIVER.

Witnesses:

H. B. BROWNELL,  
E. E. MORSE.